

## UNITED STATES PATENT OFFICE.

WILLIAM J. LAWRENCE, OF KALAMAZOO, MICHIGAN.

## PAPER-COATING MATERIAL AND PROCESS OF MAKING.

No Drawing.

Application filed December 18, 1922. Serial No. 607,700.

*To all whom it may concern:*

Be it known that I, WILLIAM J. LAWRENCE, a citizen of the United States, residing at the city and county of Kalamazoo, State of Michigan, have invented certain new and useful Improvements in Paper-Coating Materials and Processes of Making, of which the following is a specification.

1. This invention relates to improvements in paper coating material and process of making.

The objects of the invention are:

First, to provide an improved coating material which is highly colloidal and may be applied to the paper in a more concentrated form than is usual with coating material such as "satin white", thus increasing the weight of the coating which may be applied 20 at one treatment of the paper and lowering the drying cost of the same.

Second, to provide an improved coating material which does not coagulate the adhesive, such as casein size, used as a binder, 25 and does not cause the tinting or coloring to fade where it is added to the coating solution.

Third, to provide an improved coating material which may be used with good results in the production of dull finish coated papers as well as with high luster coated papers and the color of which is not affected by calendering.

Fourth, to provide an improved coating material which results in a smooth, even surface, which is desirable for printing and lithograph work.

Fifth, to provide an improved coating material which results in paper which is not readily broken or cracked in folding or bending.

I am aware that lime has been used or has entered into the manufacture of "satin white" and similar coating compositions 45 but, so far as I have observed, the result has been a harsh, unstable coating composition. While the base of my composition is lime I treat the same so that I secure a coating material which is highly colloidal, 50 is very finely divided and may be mixed with water and other coating ingredients and with less agitation than materials of the class of "satin white" now employed.

In the preparation of my improved coating composition I combine carbon dioxide

or carbonic acid gas with lime, preferably by passing carbon gas through a solution of milk of lime, after which the product may be concentrated, filtered, and pressed or dried for handling and shipment or 60 storage.

To the carbonated lime or calcium carbonate thus produced I preferably add aluminum hydroxide or its equivalent in the proportion of 40% of the alumina to 65 60% of the lime, the object of the alumina being to add luster when the coating is applied to a paper and calendered. The proportions mentioned contemplate dry weight but may, however, be very greatly varied 70 with desirable results. Adhesive such as casein size or glue or such other materials as are used in sizing may be added.

My improved coating material does not coagulate the size used as a binder or adhesive. It is an entirely neutral product and does not cause the tinting colors to change or fade where the tinting colors are added to the coating solution.

My improved coating material is adapted 80 for dull finish and also for high luster coated papers and, on account of the finely divided and highly colloidal properties, the paper coated has a very smooth, even surface, the coating being evenly distributed 85 over the entire surface.

Further, the paper coated with my improved material does not blacken or darken on calendering as is the case with certain coating materials now very generally used. 90

A still further advantage is that the paper treated or coated with my improved coating material has superior folding qualities, that is, it is not likely to crack or break on folding and because of the very 95 smooth, even surface obtained the paper is very desirable for fine printing and lithograph work.

Having thus described my invention, what I claim as new and desire to secure by Letters Patent, is:

1. The method of preparing a paper coating composition consisting of carbonating lime by passing carbon dioxide through milk of lime and mixing the calcium carbonate thus produced with aluminum hydroxide in the proportions of 60% of the calcium carbonate and 40% of the aluminum hydroxide, dry weight, and adding casein size.

2. The method of preparing a paper coat-

ing composition consisting of carbonating lime by passing carbon dioxide through milk of lime and mixing the calcium carbonate thus produced with aluminum hydroxide in the proportions of 60% of the calcium carbonate and 40% of the aluminum hydroxide, dry weight.

3. The method of preparing a paper coating composition consisting of carbonating lime by passing carbon dioxide through milk of lime and mixing the calcium carbonate thus produced with aluminum hydroxide, and adding casein size.

4. A paper coating composition comprising calcium carbonate formed by the passing of carbon dioxide through milk of lime, aluminum hydroxide, and an adhesive.

5. A paper coating composition comprising calcium carbonate formed by the pass-

ing of carbon dioxide through milk of lime, and aluminum hydroxide.

6. A paper coating composition comprising approximately 60% of calcium carbonate, 40% of aluminum hydroxide, and an adhesive. 25

7. A paper coating composition comprising approximately 60% of calcium carbonate, and 40% of aluminum hydroxide.

8. A paper coating composition comprising calcium carbonate, aluminum hydroxide, 30 and an adhesive.

9. A paper coating composition comprising calcium carbonate and aluminum hydroxide.

In witness whereof, I have hereunto set 35 my hand and seal.

WILLIAM J. LAWRENCE. [L.S.]